



US007704288B2

(12) **United States Patent**  
**Rivas et al.**

(10) **Patent No.:** **US 7,704,288 B2**  
(b5) **Date of Patent:** **\*Apr. 27, 2010**

(54) **WATER IN HYDROCARBON EMULSION USEFUL AS LOW EMISSION FUEL AND METHOD FOR FORMING SAME**

(75) Inventors: **Hercilio Rivas**, Caracas (VE); **Xiomara Gutierrez**, Caracas (VE); **Manuel A. Gonzalez**, Caracas (VE); **Geoffrey McGrath**, Caracas (VE); **Midgalia Carrasquero**, Miranda (VE); **Francisco Lopez-Linares**, San Antonio de Los Altos (VE); **Roberto Galiasso**, San Antonio de Los Altos (VE)

(73) Assignee: **Intevep, S.A.**, Caracas (VE)

(\*) Notice: Subject to any disclaimer, the term of this patent is extended or adjusted under 35 U.S.C. 154(b) by 239 days.

This patent is subject to a terminal disclaimer.

(21) Appl. No.: **11/846,283**

(22) Filed: **Aug. 28, 2007**

(65) **Prior Publication Data**

US 2008/0060258 A1 Mar. 13, 2008

**Related U.S. Application Data**

(63) Continuation of application No. 09/565,556, filed on May 5, 2000, now Pat. No. 7,276,093.

(51) **Int. Cl.**  
**C10L 1/32** (2006.01)

(52) **U.S. Cl.** ..... **44/301; 44/302**  
(58) **Field of Classification Search** ..... **44/301, 44/302**

See application file for complete search history.

(56) **References Cited**

**U.S. PATENT DOCUMENTS**

4,565,548 A 1/1986 Davis et al.

|               |        |                     |
|---------------|--------|---------------------|
| 4,568,354 A   | 2/1986 | Davis et al.        |
| 4,568,355 A   | 2/1986 | Davis et al.        |
| 4,568,356 A   | 2/1986 | Chambers            |
| 4,599,088 A   | 7/1986 | Davis et al.        |
| 4,696,638 A * | 9/1987 | DenHerder .....     |
| 4,744,796 A   | 5/1988 | Hazbun et al.       |
| 4,770,670 A   | 9/1988 | Hazbun et al.       |
| 4,908,154 A * | 3/1990 | Cook et al. .....   |
| 5,004,479 A * | 4/1991 | Schon et al. .....  |
| 5,104,418 A   | 4/1992 | Genova et al.       |
| RE35,237 E    | 5/1996 | Gunnerman           |
| 5,743,922 A   | 4/1998 | Peter-Hoblyn et al. |
| 5,873,916 A   | 2/1999 | Cemenska et al.     |

**FOREIGN PATENT DOCUMENTS**

EP 0157684 A 10/1985

(Continued)

**OTHER PUBLICATIONS**

McCutcheon's Emulsifiers and Detergents, 1983, MC Publishing Co., NJ, North American Edition, pp. 272-299.\*

McCutcheon's Emulsifiers & Detergents, 1983 North American Edition, McCutcheon Division, MC Publishing Co., Glen Rock, NJ, US, pp. 272-299.

Synthesis and centane improver performance of fatty acid glycol nitrates, G.J. Suppes et al., University of Kansas, Department of Chemical and Petroleum Engineering, Lawrence, Kansas, US, Received Dec. 5, 1997; received in revised form Jun. 24, 1998.

(Continued)

**Primary Examiner**—Cephia D Toomer

(74) **Attorney, Agent, or Firm**—Bachman & LaPointe, P.C.

(57) **ABSTRACT**

A water-in-hydrocarbon emulsion includes a water phase, a hydrocarbon phase and a surfactant, wherein the water phase is present in an amount greater than or equal to about 5% vol. with respect to volume of the emulsion, and the water phase and the surfactant are present at a ratio by volume of the water phase to the surfactant of at least about 1. A method for preparing the emulsion is also provided.

**12 Claims, 4 Drawing Sheets**



FOREIGN PATENT DOCUMENTS

|    |          |    |         |
|----|----------|----|---------|
| EP | 0157684  | A1 | 10/1985 |
| EP | 0475620  | A2 | 3/1992  |
| EP | 1252270  | A  | 10/2002 |
| GB | 2217229  | A  | 10/1989 |
| WO | 97/34969 |    | 9/1997  |
| WO | 9734969  | A1 | 9/1997  |
| WO | 9913031  | A1 | 3/1999  |
| WO | 99/35215 | A2 | 7/1999  |

WO

0148123 A1 7/2001

OTHER PUBLICATIONS

Suppes G J et al: "Synthesis and cetane improver performance of fatty acid glycol nitrates" Fuel, IPC Science and Technology Press, Guildford, GB, vol. 78, No. 1, January 1999, pp. 73-81, XP004285945 ISSN: 0016-2361.

\* cited by examiner



FIG. 1

Cylinder pressure vs crankangle. (1600 rpm/157.5 lbf-ft)



FIG. 2



FIG. 3

**FIG. 4****FIG. 5**



FIG. 6

**WATER IN HYDROCARBON EMULSION  
USEFUL AS LOW EMISSION FUEL AND  
METHOD FOR FORMING SAME**

CROSS REFERENCE TO RELATED  
APPLICATION

This is a continuation of U.S. application Ser. No. 09/565, 556, filed May 5, 2000 now U.S. Pat. No. 7,276,093.

BACKGROUND OF THE INVENTION

The invention relates to a water-in-hydrocarbon emulsion which is useful as a low emission fuel for compression ignition engines and to a method for forming same.

The impact of incorporating water into the combustion systems of Diesel engines has been presented in technical literature with an important incidence in reduction in exhaust emission rates of nitrogen oxides and particulates and with moderate reductions, and in certain cases with increases, in the exhaust emission rates of hydrocarbons and carbon monoxide. According to various investigations, the effect of reducing peak flame temperatures in the combustion chamber is the dominant cause for lower nitrogen oxide emissions.

The Clean Air Act mandates progressive decreases in smoke, particulate and nitrogen oxide emissions from both stationary and mobile sources. Attempts to address these requirements using water-in-hydrocarbon emulsions have met with very serious technical and economic problems due to the short-term stability of emulsions formed having droplet sizes in the macroemulsion range, and further due to the large quantities of surfactants and cosolvents required to form emulsions having droplet sizes in the microemulsion range.

For example, U.S. Pat. Nos. 4,568,354 and 4,568,355 to Davis et al. are drawn to processes for converting a hazy or potentially hazy water saturated alcohol-gasoline mixture into a clear stable gasoline composition having an improved octane rating. The system so produced has a water content of no more than 1% by volume, and relatively large volumes of non-ionic surfactant are used to produce this system.

Similarly, U.S. Pat. Nos. 4,770,670 and 4,744,796 to Hazbun et al. also disclose the formation of stable microemulsions which contain large amounts of surfactant as compared to the water content.

Other efforts in this area include U.S. Pat. No. 5,104,418, WO 99/35215, U.S. Pat. No. Re. 35,237, U.S. Pat. No. 5,743, 922, WO 97/34969, U.S. Pat. No. 5,873,916 and WO 99/13031.

In spite of the disclosures in the foregoing patents, the need remains in the industry for a water-in-hydrocarbon emulsion which is suitable as a combustible fuel and which contains a desirable amount of water without the need for relatively large amounts of surfactant and/or other stabilizing agents.

It is therefore the primary object of the present invention to provide water-in-hydrocarbon emulsions which are useful as combustible fuels and which are both stable and formed using relatively small amounts of surfactant.

It is a further object of the present invention to provide a method for forming such water-in-hydrocarbon emulsions utilizing a synergistic combination of mixing energy and surfactant package blend.

It is a still further object of the present invention to provide emulsions and methods for forming such emulsions wherein additional combustion properties are incorporated into the fuel through the surfactant package.

Other objects and advantages of the present invention will be readily apparent from a consideration of the following.

SUMMARY OF THE INVENTION

In accordance with the present invention, the foregoing objects and advantages have been readily attained.

In accordance with the invention, a water-in-hydrocarbon emulsion is provided, which emulsion comprises a water phase, a hydrocarbon phase and a surfactant, wherein said water phase is present in an amount greater than or equal to about 5% vol. with respect to volume of said emulsion, and said water phase and said surfactant are present at a ratio by volume of said water phase to said surfactant of at least about 1.

Stable macroemulsions and microemulsions are provided, each having advantageous features and characteristics.

In further accordance with the invention, a method is provided for forming a water-in-hydrocarbon emulsion which method comprises the steps of providing a water phase; providing a hydrocarbon phase; providing a surfactant; mixing said water phase, said hydrocarbon phase and said surfactant in amounts sufficient to provide a water content of at least about 5% vol. with respect to said emulsion, and a ratio by volume of said water phase to said surfactant of at least about 1, wherein said mixing is carried out at a mixing intensity sufficient to form a stable emulsion of said water phase in said hydrocarbon phase.

BRIEF DESCRIPTION OF THE DRAWINGS

A detailed description of preferred embodiments of the present invention follows, with reference to the attached drawings, wherein:

FIG. 1 is a schematic representation illustrating the mechanism of the mixing process of the present invention;

FIG. 2 is a comparative illustration of cylinder pressure versus crank angle of a base fuel as compared to a water-in-hydrocarbon fuel prepared in accordance with the present invention;

FIG. 3 is a comparative illustration of NO<sub>x</sub> exhaust gas emission rates at steady state conditions for a base fuel and an emulsion in accordance with the present invention;

FIG. 4 is a comparative illustration of cumulative carbon exhaust gas emission during engine transient operation utilizing a base fuel and an emulsion in accordance with the present invention;

FIG. 5 is a comparative illustration of exhaust gas peak opacity during free acceleration for a base fuel and an emulsion in accordance with the present invention; and

FIG. 6 is an illustration of interfacial tension versus concentration of monoethanolamine and the expected characteristics of the interface depending upon same.

DETAILED DESCRIPTION

The invention relates to water-in-hydrocarbon emulsions and a method for forming same whereby the emulsion is stable and can advantageously be used as a combustible fuel, for example for compression ignition engines and the like. The emulsion has beneficial characteristics as a fuel including reduced emissions. The emulsions in accordance with the present invention include stable macroemulsions and microemulsions, each of which include a dispersed water phase and a continuous hydrocarbon phase as well as an advantageous surfactant package which, as will be discussed below, is pref-

erably selected in combination with particular emulsion formation mixing intensities, so as to provide the desired stable emulsion.

Suitable hydrocarbons for use in making the emulsions of the present invention include petroleum hydrocarbons and natural gas derived products, examples of which include Diesel fuel and other low gravity hydrocarbons such as Fischer-Tropsch synthetic Diesel and paraffins C<sub>10</sub> to C<sub>20</sub>.

Emulsions including this hydrocarbon in accordance with the present invention have reduced NO<sub>x</sub> emissions and C emissions, and improved opacity as compared to the hydrocarbon alone.

Further, improvement in air-fuel mixing conditions and of evaporative spray in the combustion chamber of Diesel engines can be accomplished utilizing the emulsion as compared to the base fuel, which can result in improvements in the fuel fraction efficiency and a better energy balance utilization in combination with the lower exhaust gas and particulate emissions. One example of a suitable hydrocarbon is a Diesel fuel characterized as follows:

TABLE 1

|                    |                      |      |
|--------------------|----------------------|------|
| Sulfur content     | (% wt/wt)            | <0.5 |
| Density @ 15° C.   | (kg/m <sup>3</sup> ) | <860 |
| Viscosity @ 40° C. | (mm <sup>2</sup> /s) | <4.5 |
| T95                | (° C.)               | <370 |
| Flash point        | (° C.)               | >52  |

The water phase for use in forming emulsions in accordance with the present invention can suitably be from any acceptable water source, and is preferably a water which is available in sufficient quantities, preferably in close proximity to the location where emulsions are to be formed, and preferably at an inexpensive cost. For example, a suitable water phase could be water such as 310 ppm brine. Of course, any other water from a suitable source and having various acceptable characteristics for use as a component of a combustible fuel would be acceptable.

The surfactant package forms an important portion of the present invention, particularly when combined with particular emulsion forming steps as will be further described below. The surfactant or surfactant package of the present invention is preferably a package including both a lipophilic surfactant component and a hydrophilic surfactant component. This combination of components advantageously serves to increase the amount of molecules which are present at the water-hydrocarbon interface, and to minimize the interfacial tension therein, thereby allowing substantially reduced amounts of surfactants to be utilized while nevertheless providing a stable emulsion. This is particularly advantageous from a cost standpoint as compared to conventional known emulsions and processes.

Suitable surfactants, as set forth above, include both lipophilic surfactant components and hydrophilic surfactant components. Suitable lipophilic surfactant components include neat oleic acid, sorbitan ester monooleate, sorbitan ester trioleate, ethoxylated oleic acid and mixtures thereof. These lipophilic surfactant components typically have a hydrophilic-lipophile balance, or HLB, of between about 1 and about 8. The hydrophilic-lipophile balance or HLB of a surfactant is the relative simultaneous attraction that the surfactant demonstrates for water and oil. Substances having a high HLB, above about 12, are highly hydrophilic while substances having a low HLB, below about 8, are highly lipophilic. Surfactants having an HLB between about 8 and about 12 are considered intermediate.

Suitable hydrophilic surfactant components include oleic acid which has been neutralized, preferably 100% neutralized, with monoethanolamine, polyethoxylated fatty amine and mixtures thereof. These hydrophilic surfactant components typically have an HLB of between about 10 and about 18.

Neutralized oleic acid may be formed as hydrophilic surfactant component by mixing, either separately or during emulsion formation, neat oleic acid and monoethanolamine (MEA) whereby oleate ions are formed as further discussed below.

Additional components such as cosolvents for microemulsions, and other additives, may also be present.

As will be discussed more thoroughly below in connection with the process for forming the emulsion, surfactant components which are both lipophilic and hydrophilic are preferably selected and mixed for use in forming the emulsion, and this advantageously results in the formation of an interface in the emulsion between the water phase and the hydrocarbon phase which includes a mixture of both surfactant components.

Microemulsions according to the invention are advantageously provided with a ratio by volume of water to surfactant which is greater than about 1. Macroemulsions according to the invention are advantageously formed with very small amounts of surfactant, preferably less than or equal to about 4% vol., and having a ratio by volume of water to surfactant of greater than about 2.5.

The emulsions of the present invention preferably include water by volume with respect to the emulsion in an amount of at least about 5%, preferably between about 5% vol. and about 15% vol. with respect to total volume of the emulsions. As will be illustrated in the data to follow, the particular surfactant package and the mixing intensity or energy dissipation rate of the present invention both appear critical in providing acceptably stable emulsions.

It should also be noted that the emulsion of the present invention as compared to a base fuel from which the emulsion was prepared compares favorably in connection with engine cylinder pressure versus crank angle, NO<sub>x</sub> exhaust gas emission, carbon exhaust gas emission, exhaust gas peak opacity and the like.

As set forth above, it is also within the scope of the present invention to modify the surfactant package so as to include additional functional groups which can be selected so as to provide desirable properties in the resulting emulsion fuel.

For example, a nitro-olefin derivate of oleic acid can be obtained, for example by using nitrogen monoxide to modify the oleic acid. Such a nitro-olefin derivate of oleic acid can be utilized during emulsion formation and remains active in the final emulsion as a cetane number improver for providing the emulsion with a higher cetane number as compared to a microemulsion formed with a normal oleic acid as a component of the surfactant package. Of course, other functional groups, particularly other nitrogen functional groups, could advantageously be incorporated into the surfactant package for various other desirable results. Other functional groups that can advantageously be incorporated into the surfactant package include ketones, hydroxy and epoxy groups, and the like.

Emulsions in accordance with the present invention may suitably be formed as described below.

Suitable supplies of both water phase and hydrocarbon phase are obtained.

Once it is determined what type of emulsion is desired, that is, a microemulsion or a macroemulsion, a suitable surfactant package is selected.

## 5

Referring to FIG. 1, the steps of the method of the present invention are illustrated in terms of the type of droplet size formed and status of the surfactant. The process preferably starts the formation of a coarse dispersion which is refined and homogenized by turbulence-length scales of decreasing size (through mixing mechanisms associated with turbulent diffusion). The final stage of mixing involves microscale engulfment and stretching where the ultra low surface tension results in the formation of a microemulsion. Where no ultra-low interfacial tension is achieved, the fineness of the dispersion, for a given surfactant package, depends upon the intensity of the turbulence.

In order to prepare a microemulsion, the surfactant package is preferably selected including a hydrophilic component and a lipophilic component which are balanced so as to provide a surfactant package HLB of between about 6 and about 10. This surfactant package will be acceptable when utilized in conjunction with the additional process steps of the present invention for providing a stable microemulsion.

In order to form a suitable microemulsion, the three components, that is, the water phase, hydrocarbon phase and surfactant package are preferably combined in the desired volumes and subjected to a mixing intensity (W/kg) which is selected in accordance with the present invention in order to provide the desired type of emulsion. In accordance with the invention, to form a microemulsion, it is desirable to utilize a surfactant package having an HLB between about 6 and about 10 and a mixing intensity of between about 1 W/kg and about 10,000 W/kg. On an in-line production scale, the mixing intensity is more preferably between about 100 and about 1000 W/kg. If production rates are not critical, average mixing intensities between about 1 W/kg and about 100 W/kg also provide a stable microemulsion. Mixing according to the invention advantageously results in a desirable stable microemulsion having an average droplet size of between about 100 Å and about 700 Å. Emulsions formed according to the invention are advantageously stable in that the emulsion will retain an average droplet diameter, when stored under normal ambient conditions, for at least about 1 year and typically for an indefinite period of time.

The mixing intensity referred to herein is presented as average mixing intensity, averaged over the mixing profile of a vessel. Depending upon the mixing intensity and mixing time used, different orders of mixing intensity can be encountered within the mixing vessel. For example, mixing can be accomplished in accordance with the present invention utilizing a Rushton impulson coupled to a Heidolph motor for providing the desired mechanical energy dissipation rate or mixing intensity. In a typical vessel mixed with this equipment, while the vessel may be mixed having an average energy dissipation rate of about 1 W/kg, the mixing intensity in close proximity to the mixing apparatus can in actuality be closer to the order of 100 W/kg. Mixing under such conditions will be referred to herein as mixing at an average mixing intensity of about 1 W/kg, or in the alternative, as 1-100 W/kg.

With other equipment, such as a rotor-stator mixer, the mixing intensity can be made nearly uniform.

It should also be noted that the mixing intensity as referred to herein relates to the energy dissipation rate as measured in power dissipated per unit mass of liquid in the mixer. The flow is assumed to be turbulent.

## 6

The different phases used for forming the microemulsion are preferably mixed so as to provide a water content in the final emulsion of at least about 5%, preferably between about 5% vol. and about 15% vol. with respect to total volume of the final emulsion product. The surfactant package is preferably provided in amounts of less than or equal to about 14% vol. with respect to the emulsion, which is particularly advantageous as compared to the amounts of surfactant package required to provide a stable microemulsion using conventional techniques. It is particularly advantageous that the method of the present invention allows for preparation of an emulsion having a ratio by volume of water to surfactant package which is greater than or equal to about 1.

In order to form a suitably stable microemulsion, it may also be necessary to utilize a small volume of cosolvent. However, it should be noted that the amount of cosolvent necessary is substantially reduced as compared to conventional processes as well. Typically, a suitably stable microemulsion can be formed utilizing less than or equal to about 2% vol. of cosolvent. Suitable cosolvents are alcohols, preferably an alcohol selected from the group consisting of methanol, ethanol, iso-propanol, n-butanol, ter-butanol, n-pentanol, n-hexanol and mixtures thereof.

In accordance with the present invention, it is preferred to mix the surfactant package and the cosolvent with the hydrocarbon phase, and then to mix the water and hydrocarbon phases together. Of course, other mixing procedures are also suitable within the scope of the present invention.

Suitable mixing equipment is readily available to the person of ordinary skill in the art. Examples of suitable mixing equipment are set forth above and in the examples to follow.

It should also be noted that various additional additives can be incorporated into the emulsion depending upon desired characteristics and intended use of the final emulsion product.

As set forth above, the surfactant package can advantageously be modified so as to include performance improving functional groups such as nitro-groups and the like which advantageously serve to improve the cetane number of the final emulsion product.

Macroemulsions are formed in accordance with the present invention as follows. As with microemulsion preparation supplies of suitable water and hydrocarbon phases are obtained.

A surfactant package is then preferably selected having an HLB of between about 3 and about 10. As with the microemulsions, this HLB is obtained by blending lipophilic and hydrophilic surfactant components as described above, in proportions sufficient to provide the desired HLB. The water, hydrocarbon and surfactant package components are then mixed at a mixing intensity selected so as to provide the desired macroemulsion, preferably having an average droplet size of between about 0.5 and about 2.0 microns. It is preferred that the macroemulsion be mixed at a mixing intensity of greater than or equal to about 10,000 W/kg, and this mixing intensity corresponds to an energy dissipation rate during turbulent flow as with the microemulsion formation process. The acceptable mixing intensity can be imparted to the mixture of ingredients using known equipment which would be readily available to the person of ordinary skill in the art.

Macroemulsions can advantageously be formed in accordance with the method of the present invention without the need for cosolvents which are typically required to form macroemulsions according to conventional procedures. Thus,

the surfactant stabilizing portion of the emulsion and surfactant package preferably consists essentially of the lipophilic surfactant component and the hydrophilic surfactant component, and the emulsion can be prepared substantially free of any cosolvents whatsoever. This is particularly advantageous in reducing the cost of the final product.

As will be set forth in the samples to follow, water in hydrocarbon emulsions prepared in accordance with the present invention clearly compare favorably to the base hydrocarbon when used as a fuel and show consistent reduction in  $\text{NO}_x$  and other favorable properties as compared to the base fuel.

The following examples demonstrate advantageous characteristics of the emulsions of the present invention.

#### EXAMPLE 1

This example illustrates the formation of microemulsions in accordance with the present invention and demonstrates the criticality of mixing intensity or energy dissipation rate in providing a stable microemulsion using reduced amounts of surfactants. Values provided in this example will be average mixing intensities based on total mass of mixture. It should of course be noted that mixing intensities much larger than average can be encountered in the mixing vessel, for example near the mixing apparatus.

Microemulsions were prepared utilizing 5% volume of water (310 ppm brine), a hydrocarbon phase of Diesel fuel as described above in Table 1 and surfactant packages including one or more components of lipophilic neat oleic acid (HLB=1.3), lipophilic sorbitan ester monooleate (HLB=4.3) and lipophilic ethoxylated oleic acid (5 EO, HLB=7.7), and hydrophilic oleic acid 100% neutralized with monoethanolamine.

The first samples of emulsion prepared under this example were prepared using a surfactant package including a lipophilic surfactant component of oleic acid having an HLB of 1.3 and a hydrophilic oleic acid 100% neutralized with monoethanolamine (oleate ions, HLB=18). These components were provided in a 1:1 ratio by volume and utilized to form emulsions as set forth in Table 2 below:

Sample 1 was prepared using 8% volume of surfactant package and a mixing intensity generated through manual agitation of about 0.1 W/kg or less for approximately 2-5 minutes (spontaneous formation). Sample 2 was prepared utilizing 4% volume of surfactant package and moderate turbulence utilizing a Rushton impulsor coupled to a Heidolph motor for providing an average mechanical energy dissipation rate of 1 W/kg for a period of approximately 5 minutes. Sample 3 was prepared also utilizing 4% volume of the surfactant package, but with manual agitation of less than 0.1 W/kg as with Sample 1.

15

As shown in Table 2, Sample 1 resulted in a microemulsion, but required 8% volume of surfactant. Sample 3 utilizing 4% volume of the surfactant package and manual agitation resulted in an unstable macroemulsion.

Sample 2, prepared in accordance with the present invention, provided a stable microemulsion utilizing only 4% volume of surfactant package which is, of course, advantageous as compared to the 8% volume required for Sample 1.

25

Samples 4-5 were then prepared utilizing the same surfactant package and 10% volume of water. Sample 4 was prepared utilizing 14% volume of surfactant package and manual agitation. Sample 5 was prepared using 7% volume of surfactant package and a vessel averaged mixing intensity of 1 W/kg. Sample 6 was prepared utilizing 7% volume of surfactant package and manual agitation.

30

Table 3 sets forth the results obtained for these samples.

TABLE 2

| Sample No. | Surfactant                                                        | Vol. % Diesel | Vol. % Surfactant | Vol. % Monoethanolamine | Vol. % Deionized Water (310 ppm Brine) | Vol. % n-Hexanol | HLB | Mixing Intensity W/kg | Obs.                    |
|------------|-------------------------------------------------------------------|---------------|-------------------|-------------------------|----------------------------------------|------------------|-----|-----------------------|-------------------------|
| 1          | Neat Oleic Acid/Oleic Acid 100% neutralized with monoethanolamine | 84.6          | 8 (4/4)           | 0.86                    | 5                                      | 1.5              | 9.5 | Manual agitation      | Micro-emulsion          |
| 2          | Neat Oleic Acid/Oleic Acid 100% neutralized with monoethanolamine | 89.1          | 4 (2/2)           | 0.43                    | 5                                      | 1.5              | 9.5 | 1                     | Micro-emulsion          |
| 3          | Neat Oleic Acid/Oleic Acid 100% neutralized with monoethanolamine | 89.1          | 4 (2/2)           | 0.43                    | 5                                      | 1.5              | 9.5 | Manual agitation      | Unstable Macro-emulsion |

TABLE 3

| Sample No. | Surfactant                                                        | Vol. % Diesel | Vol. % Surfactant | Vol. % Monoethanolamine | Vol. % Deionized Water (310 ppm Brine) | Vol. % n-Hexanol | HLB | Mixing Intensity W/Kg | Obs.                   |
|------------|-------------------------------------------------------------------|---------------|-------------------|-------------------------|----------------------------------------|------------------|-----|-----------------------|------------------------|
| 4          | Neat Oleic Acid/Oleic Acid 100% neutralized with monoethanolamine | 73.6          | 14 (7.6/6.4)      | 1.40                    | 10                                     | 1.0              | 8.9 | Manual agitation      | Microemulsion          |
| 5          | Neat Oleic Acid/Oleic Acid 100% neutralized with monoethanolamine | 81.3          | 7 (3.8/3.2)       | 0.70                    | 10                                     | 1.0              | 8.9 | 1                     | Microemulsion          |
| 6          | Neat Oleic Acid/Oleic Acid 100% neutralized with monoethanolamine | 81.3          | 4 (3.8/3.2)       | 0.70                    | 10                                     | 1.0              | 8.9 | Manual agitation      | Unstable Macroemulsion |

As shown, Sample 4 resulted in a microemulsion, but required 14% volume of surfactant, which is greater than the water content of this emulsion. Sample 6 utilizing a lower content of surfactant resulted in an unstable macroemulsion.

Sample 5 prepared in accordance with the present invention resulted in a stable microemulsion while advantageously utilizing a substantially reduced amount of surfactant package as compared to Sample 4.

It should be noted that an additional sample was prepared utilizing the same amounts of components as listed for Sample 5, but with mixing intensity increased to 10,000 W/kg, and a stable microemulsion resulted. Here, a rotor-

stator mixer was used and so the intensities of mixing can be made nearly uniform resulting in a single intensity value.

Samples 7-9 were prepared utilizing the same surfactant package discussed above with water content of 15% volume. Sample 7 was prepared using 20% volume of the surfactant package and manual agitation, Sample 8 was prepared in a conventional stirrer (Rushton disc turbine) utilizing 14% volume of surfactant package and moderate vessel-averaged mixing intensity of 1 W/kg, and Sample 9 was prepared utilizing 14% volume surfactant package and manual agitation. The results are set forth in Table 4.

TABLE 4

| Sample No. | Surfactant                                                        | Vol. % Diesel | Vol. % Surfactant | Vol. % Monoethanolamine | Vol. % Deionized Water (310 ppm Brine) | Vol. % n-Hexanol | HLB | Mixing Intensity W/Kg | Obs.                   |
|------------|-------------------------------------------------------------------|---------------|-------------------|-------------------------|----------------------------------------|------------------|-----|-----------------------|------------------------|
| 7          | Neat Oleic Acid/Oleic Acid 100% neutralized with monoethanolamine | 61.3          | 20 (10/10)        | 2.15                    | 15                                     | 1.5              | 9.5 | Manual agitation      | Microemulsion          |
| 8          | Neat Oleic Acid/Oleic Acid 100% neutralized with monoethanolamine | 68            | 14 (7/7)          | 1.51                    | 15                                     | 1.5              | 9.5 | 1                     | Microemulsion          |
| 9          | Neat Oleic Acid/Oleic Acid 100% neutralized with monoethanolamine | 68            | 14 (7/7)          | 1.51                    | 15                                     | 1.5              | 9.5 | Manual agitation      | Unstable Macroemulsion |

## 11

As shown, Sample 7 resulted in a stable microemulsion, but required more surfactant than water was present. Sample 9 utilized less surfactant package, but resulted in an unstable macroemulsion.

Sample 8, prepared in accordance with the present invention, provided a stable microemulsion having a ratio of water to surfactant of greater than 1.

Samples 10-12 were prepared utilizing a surfactant package including lipophilic sorbitan ester monooleate having an HLB of 4.3 and neat oleic having HLB equal to 1.3, and

## 12

hydrophilic oleic acid which has been 100% neutralized with monoethanolamine (oleate ions, HLB=18). Samples 10 and 12 were prepared utilizing manual agitation for 2-5 minutes ( $\leq 0.1$  W/kg). Sample 11 was prepared utilizing moderate turbulence, for approximately 1.5 minutes, while mixing with a Rushton impulser coupled to a Heidolph motor which provided a vessel averaged mechanical energy of 1 W/kg.

The results are shown in Table 5 for 10% volume water emulsions.

TABLE 5

| Sample No. | Surfactant                                                                                       | Vol. % Diesel | Vol. % Surfactant | Vol. % Mono-ethanol-amine | Vol. % Deionized Water (310 ppm Brine) | Vol. % n-Hexanol | HLB | Mix. Inten. W/Kg | Obs.                    |
|------------|--------------------------------------------------------------------------------------------------|---------------|-------------------|---------------------------|----------------------------------------|------------------|-----|------------------|-------------------------|
| 10         | Sorbitan ester monooleate/<br>Neat Oleic Acid/Oleic Acid, 100% neutralized with Monoethanolamine | 73            | 13<br>(5.1/3/4.9) | 1.04                      | 10                                     | 3.0              | 9.3 | Man agit.        | Micro-emulsion          |
| 11         | Sorbitan ester monooleate/<br>Neat Oleic Acid/Oleic Acid, 100% neutralized with Monoethanolamine | 81.6          | 5<br>(2/1.1/1.9)  | 0.4                       | 10                                     | 3.0              | 9.3 | 1                | Micro-emulsion          |
| 12         | Sorbitan ester monooleate/<br>Neat Oleic Acid/Oleic Acid, 100% neutralized with Monoethanolamine | 81.6          | 5<br>(2/1.1/1.9)  | 0.4                       | 10                                     | 3.0              | 9.3 | Man. agit.       | Unstable Macro-emulsion |

Sample 10 included 13% volume of the surfactant package and was made using manual agitation, and resulted in a microemulsion. However, this emulsion has a ratio of water to surfactant package of less than 1. Sample 12 was prepared using 5% volume of the surfactant package and manual agitation, but resulted in an unstable macroemulsion. Sample 11 prepared in accordance with the present invention utilized 5% volume of the surfactant package and moderate turbulence and resulted in a stable microemulsion as desired.

Samples 13-15 were then prepared utilizing a surfactant system including lipophilic ethoxylated oleic acid (5 EO, HLB=7.7), and oleic acid 100% neutralized with monoethanolamine (oleate ions, HLB=18).

Samples 13-15 were prepared using 10% volume of water. Sample 13 was prepared utilizing 15% volume of surfactant package and manual agitation. Sample 15 was prepared utilizing 10% volume surfactant package and manual agitation and Sample 14 was prepared with a Rushton disc turbine utilizing 10% of the surfactant package and moderate vessel-average turbulence intensity of 1 W/kg. Table 6 sets forth the results.

TABLE 6

| Sample No. | Surfactant                                                                       | Vol. % Diesel | Vol. % Surfactant | Vol. % Monoethanolamine | Vol. % Deionized Water (310 ppm Brine) | Vol. % n-Hexanol | HLB | Mix. Inten. W/Kg | Obs.                    |
|------------|----------------------------------------------------------------------------------|---------------|-------------------|-------------------------|----------------------------------------|------------------|-----|------------------|-------------------------|
| 13         | Ethoxylated Oleic Acid (5 EO)/Oleic Acid, 100% neutralized with Monoethanolamine | 66.4          | 15 (12/3)         | 0.65                    | 10                                     | 8.0              | 9.8 | Man. agit.       | Micro-emulsion          |
| 14         | Ethoxylated Oleic Acid (5 EO)/Oleic Acid, 100% neutralized with Monoethanolamine | 75.6          | 10 (8/2)          | 0.43                    | 10                                     | 4.0              | 9.8 | 1                | Micro-emulsion          |
| 15         | Ethoxylated Oleic Acid (5 EO)/Oleic Acid, 100% neutralized with Monoethanolamine | 75.6          | 10 (8/2)          | 0.43                    | 10                                     | 4.0              | 9.8 | Man. agit.       | Unstable Macro-emulsion |

Sample 13 resulted in a stable microemulsion, but required 15% volume surfactant which is greater than the water content of the emulsion. Sample 15 utilized less surfactant, but resulted in an unstable macroemulsion at the manual agitation. Sample 14 prepared in accordance with the present invention resulted in a stable microemulsion advantageously having a ratio by volume of water to surfactant 1.

It is clear from the results illustrated in Table 2-6 that the mixing intensity of the present invention is critical in allowing reduction of the surfactant package concentration used while forming a stable microemulsion, and that the method of the present invention readily provides stable microemulsions having water to surfactant ratio by volume of greater than 1 or equal to.

## EXAMPLE 2

30 This example demonstrates the criticality of the desired HLB of the surfactant package in accordance with the present invention.

In this example, emulsions are formed using Diesel fuel as in Example 1 and using water phase of water (310 ppm brine) in the amount of 10% volume with respect to the emulsion. 35 Each emulsion has been formed utilizing equipment as described in Example 1 to provide average mixing intensity or energy dissipation rate per unit mass of about 1 W/kg, with local intensities of about 100 W/kg.

The surfactant package in this example will include one or 40 more surfactant components of lipophilic neat oleic acid, sorbitan ester monooleate, and sorbitan ester trioleate, and hydrophilic oleic acid neutralized with monoethanolamine and polyethoxylated fatty amine (5 NOE).

Table 7 sets forth results obtained for Samples 1-6—prepared using different surfactant packages as listed in the table.

TABLE 7

| Sample No. | Surfactant                                                           | Vol. % Diesel | Vol. % Surfactant | Vol. % Monoethanolamine | Vol. % Deionized Water (310 ppm Brine) | Vol. % n-Hexanol | HLB  | Mix. Inten. W/Kg | Obs.                        |
|------------|----------------------------------------------------------------------|---------------|-------------------|-------------------------|----------------------------------------|------------------|------|------------------|-----------------------------|
| 1          | Neat Oleic Acid                                                      | 82.0          | 7                 | 0                       | 10                                     | 1.0              | 1.03 | 1                | Two distinct liquid phases  |
| 2          | Oleic Acid, 100% neutralized with Monoethanolamine                   | 80.5          | 7                 | 1.52                    | 10                                     | 1.0              | 18.0 | 1                | Oil in water Macro-emulsion |
| 3          | Neat Oleic Acid 100% neutralized with Monoethanolamine (oleate ions) | 81.3          | 7 (3.8/3.2)       | 0.7                     | 10                                     | 1.0              | 8.9  | 1                | Micro-emulsion              |

## 15

As shown, Sample 1 was prepared utilizing only neat oleic acid having an HLB of 1.03, and two distinct liquid phases were obtained. Sample 2 was prepared utilizing only oleic acid 100% neutralized with monoethanolamine, such that the surfactant package has an HLB of 18.0, and an undesirable oil-in-water macroemulsion resulted. Sample 3, prepared uti-

## 16

lizing a surfactant package including 3.8% volume neat oleic acid and 3.2% volume oleic acid 100% neutralized with monoethanolamine resulted in a surfactant package having an HLB of 8.9 and provided a desirable stable microemulsion.

Table 8 sets forth compositions utilized to prepare Samples 4-6 and results obtained.

TABLE 8

| Sample No. | Surfactant                                            | Vol. % Diesel | Vol. % Surfactant | Vol. % Monoethanol-amine | Vol. % Deionized Water (310 ppm Brine) | Vol. % n-Hexanol | HLB  | Mix. Inten. W/Kg | Obs.                         |
|------------|-------------------------------------------------------|---------------|-------------------|--------------------------|----------------------------------------|------------------|------|------------------|------------------------------|
| 4          | Sorbitan ester monooleate                             | 81.7          | 8.3               | 0                        | 10                                     | 0.0              | 4.3  | 1                | Unstable water in Oil Macro- |
| 5          | Polyethoxylated fatty amine                           | 81.7          | 8.3               | 0                        | 10                                     | 0.0              | 10.0 | 1                | Unstable water in Oil Macro- |
| 6          | Sorbitan ester monooleate/polyethoxylated fatty amine | 81.7          | 8.37 (6/2.3)      | 0                        | 10                                     | 0.0              | 8.3  | 1                | emulsion Micro-emulsion      |

Sample 4 was prepared utilizing only sorbitan ester monooleate as surfactant package, resulting in an HLB of 4.3 and an unstable water-oil-macroemulsion. Sample 5 was prepared using only polyethoxylated fatty amine (HLB of 10), and produced an unstable oil-in-water macroemulsion. Sample 6 was prepared utilizing 6% volume of sorbitan ester monooleate and 2.3% volume of polyethoxylated fatty amine for a resulting surfactant package HLB of 8.4. This sample produced a desirable stable microemulsion.

Table 9 sets forth results obtained for Samples 7-9.

TABLE 9

| Sample No. | Surfactant                                                                   | Vol. % Diesel | Vol. % Surfactant | Vol. % Monoethanol-amine | Vol. % Deionized Water (310 ppm Brine) | Vol. % n-Hexanol | HLB  | Mix. Inten. W/Kg | Obs.                        |
|------------|------------------------------------------------------------------------------|---------------|-------------------|--------------------------|----------------------------------------|------------------|------|------------------|-----------------------------|
| 7          | Oleic Acid, 100% neutralized with Monoethanolamine                           | 80.2          | 6                 | 1.3                      | 10                                     | 2.5              | 18.0 | 1                | Oil in water Macro-emulsion |
| 8          | Sorbitan ester trioleate                                                     | 81.5          | 6                 | 0.0                      | 10                                     | 2.5              | 1.8  | 1                | Water in Oil Macro-emulsion |
| 9          | Oleic Acid, 100% neutralized with Monoethanolamine/ Sorbitan ester trioleate | 81.07         | 6 (2/4)           | 0.43                     | 10                                     | 2.5              | 7.2  | 1                | Micro-emulsion              |

## 17

Sample 7 was prepared utilizing a surfactant package of only oleic acid 100% neutralized with monoethanolamine and having an HLB of 18.0. This resulted in an undesirable oil-in-water macroemulsion. Sample 8 was prepared utilizing only sorbitan ester trioleate as the surfactant package, resulting in an HLB of 1.8 and an undesirable water-in-oil macroemulsion. Sample 9 was prepared utilizing 2% volume of

## 18

oleic acid 100% neutralized with monoethanolamine and 4% volume sorbitan ester trioleate resulting in a surfactant package HLB of 7.2 and a desirable stable microemulsion.

5 Table 10 shows an emulsion prepared using a paraffin hydrocarbon (hexadecane) and the surfactant package in accordance with the present invention.

TABLE 10

| Sample No. | Surfactant                                                                      | Vol. % Diesel | Vol. % Surfactant | Vol. % Mono-ethanol-amine | Vol. % Deionized Water (310 ppm Brine) | Vol. % n-Hexanol | Mix. HLB | Inten. W/Kg | Obs.          |
|------------|---------------------------------------------------------------------------------|---------------|-------------------|---------------------------|----------------------------------------|------------------|----------|-------------|---------------|
| 1          | Neat Oleic Acid/Oleic Acid 100% neutralized with monoethanolamine (oleate ions) | 79.7          | 9.4 (7.1/1.9)     | 0.41                      | 10                                     | 0.5              | 4.5      | 1           | Microemulsion |

25 As shown, through utilizing a surfactant package including 7.1% volume neat oleic acid and 1.9% volume oleic acid 100% neutralized with monoethanolamine, and mixing at an average intensity of 1 W/kg, a stable microemulsion is obtained. As shown, for this microemulsion, the surfactant package is prepared so as to provide an HLB of 4.5. This is in accordance with the findings of the present invention, wherein it has been found that lower HLB values, preferably between about 2 and about 5, are required in order to form a successful stable microemulsion for paraffin hydrocarbons.

35

## EXAMPLE 3

This example illustrates the advantageously reduced amounts of solvent or cosolvent required in order to form stable microemulsions in accordance with the present invention.

40 Microemulsions having 10% volume of water and Diesel fuel as dehydrocarbon phase were prepared using various mixing intensities.

Table 11 set forth below illustrates results obtained for Samples 1-3.

TABLE 11

| Sample No. | Surfactant                                                                      | Vol. % Diesel | Vol. % Surfactant | Vol. % Mono-ethanol-amine | Vol. % Deionized Water (310 ppm Brine) | Vol. % n-Hexanol | Mix. HLB | Inten. W/Kg | Obs.                   |
|------------|---------------------------------------------------------------------------------|---------------|-------------------|---------------------------|----------------------------------------|------------------|----------|-------------|------------------------|
| 1          | Neat Oleic Acid/Oleic Acid 100% neutralized with Monoethanolamine (oleate ions) | 81.3          | 7 (3.8/3/2)       | 0.7                       | 10                                     | 1.0              | 8.9      | Man. agit.  | Unstable Macroemulsion |
| 2          | Neat Oleic Acid/Oleic Acid 100% neutralized with Monoethanolamine (oleate ions) | 77.3          | 7 (3.8/3/2)       | 0.7                       | 10                                     | 5.0              | 8.9      | Man. agit.  | Microemulsion          |

TABLE 11-continued

| Sample No. | Surfactant                                                                      | Vol. % Diesel | Vol. % Surfactant | Vol. % Monoethanolamine | Deionized Water (310 ppm Brine) | Vol. % n-Hexanol | HLB | Mix. Inten. W/Kg | Obs.          |
|------------|---------------------------------------------------------------------------------|---------------|-------------------|-------------------------|---------------------------------|------------------|-----|------------------|---------------|
| 3          | Neat Oleic Acid/Oleic Acid 100% neutralized with Monoethanolamine (oleate ions) | 81.3          | 7 (3.8/3.2)       | 0.7                     | 10                              | 1.0              | 8.9 | 1                | Microemulsion |

15

As shown in Table 11, each sample was prepared using a surfactant package having 3.8% volume neat oleic acid and 3.2% volume oleic acid 100% neutralized with monoethanolamine. Sample 1 was prepared using 1% volume of n-Hexanol cosolvent, and manual agitation of less than or equal to about 0.1 W/kg, and an unstable macroemulsion resulted.

Sample 2 was prepared using the same volume of surfactant package and 5% volume of n-Hexanol cosolvent, and manual agitation was sufficient to provide a microemulsion. Sample 3, prepared in accordance with the present invention using a conventional stirrer (Rushton disc turbine), also utilized the same volume percentage of surfactant package, and 1% volume of n-Hexanol cosolvent, with a vessel averaged mixing intensity of 1 W/kg, and a stable microemulsion resulted.

Table 12 shows results obtained for Samples 4, 5 and 6 prepared using n-butanol cosolvent.

Sample 4 was prepared with 0.8% volume n-butanol and manual agitation, and an unstable macroemulsion resulted.

20 Sample 5 was prepared using 7.0% volume n-butanol and manual agitation, and a satisfactory microemulsion resulted.

25 Sample 6 was prepared in accordance with the present invention (standard Rushton disc turbine) and contained 0.8% volume n-butanol and was mixed at a vessel-averaged mixing intensity of 1 W/kg, and a desirable stable microemulsion resulted. Thus, preparation of the emulsion in accordance with the present invention allows formation of a stable microemulsion with significantly reduced concentrations of cosolvent.

30 35 Similar results were also obtained in accordance with the present invention utilizing less than or equal to about 1% volume of n-butanol, isopropanol, ethanol and methanol cosolvents, and this is set forth in Table 13.

TABLE 12

| Sample No. | Surfactant                                                                      | Vol. % Diesel | Vol. % Surfactant | Vol. % Monoethanolamine | Deionized Water (310 ppm Brine) | Vol. % n-Butanol | HLB | Mix. Intens. W/Kg | Obs.                   |
|------------|---------------------------------------------------------------------------------|---------------|-------------------|-------------------------|---------------------------------|------------------|-----|-------------------|------------------------|
| 4          | Neat Oleic Acid/Oleic Acid 100% neutralized with Monoethanolamine (oleate ions) | 79.4          | 9                 | 0.8                     | 10                              | 0.8              | 8.0 | Man. agit.        | Unstable Macroemulsion |
| 5          | Neat Oleic Acid/Oleic Acid 100% neutralized with Monoethanolamine (oleate ions) | 73.2          | 9                 | 0.8                     | 10                              | 7.0              | 8.0 | Man. agit.        | Microemulsion          |
| 6          | Neat Oleic Acid/Oleic Acid 100% neutralized with Monoethanolamine (oleate ions) | 79.4          | 9                 | 0.8                     | 10                              | 0.8              | 8.0 | 1                 | Microemulsion          |

TABLE 13

| Cosolvent<br>(% (v/v)) | Diesel<br>% (v/v) | Oleic Acid<br>% (v/v) | Mon-<br>ethanol-<br>amine<br>% (v/v) | H <sub>2</sub> O<br>% (v/v) | HLB |
|------------------------|-------------------|-----------------------|--------------------------------------|-----------------------------|-----|
| Methanol<br>(0.2)      | 80.1              | 9                     | 0.7                                  | 10                          | 7.3 |
| Ethanol<br>(0.77)      | 79.4              | 9                     | 0.8                                  | 10                          | 8   |
| Isopropanol<br>(0.69)  | 79.6              | 9                     | 0.7                                  | 10                          | 7   |
| n-Propanol<br>(0.8)    | 79.4              | 9                     | 0.8                                  | 10                          | 8   |

Table 13 lists four separate stable microemulsions that were formed and the amount of cosolvent, hydrocarbon phase, surfactant, water and HLB for each emulsion. In each

case, a stable microemulsion is provided in each case using less than 1% volume of cosolvent and a vessel-averaged mixing intensity of 1 W/kg.

5

## EXAMPLE 4

This example illustrates preparation of macroemulsions in accordance with the present invention. These macroemulsions are in all cases water in Diesel (W/O) two phase systems, and are opaque to visible light (milky appearance).  
10 Macroemulsions are defined as emulsions having an average droplet size of between about 0.5 and about 2 microns.

The surfactant package used in preparing each of these emulsions included one or more surfactant components including lipophilic neat oleic acid, lipophilic sorbitan ester 15 monooleate and hydrophilic oleic acid 100% neutralized with monoethanolamine.

Table 14 shows results obtained for samples 1 and 2 as set forth below.

TABLE 14

| Sample<br>No. | Surfactant                                                                         | Vol. %<br>Diesel | Vol. %<br>Surfactant | Vol. %<br>Mono-<br>ethanol-<br>amine | Deionized<br>Water<br>(310 ppm<br>Brine) |     | Vol. %<br>n-Hexanol | HLB    | Mix.<br>Inten.<br>W/Kg         | Obs. |
|---------------|------------------------------------------------------------------------------------|------------------|----------------------|--------------------------------------|------------------------------------------|-----|---------------------|--------|--------------------------------|------|
|               |                                                                                    |                  |                      |                                      | 5                                        | 0.0 |                     |        |                                |      |
| 1             | Neat Oleic<br>Acid/Oleic<br>Acid 100%<br>neutralized<br>with Mono-<br>ethanolamine | 93.0             | 1<br>(0.89/0.11)     | 0.026                                | 5                                        | 0.0 | 3.0                 | 1      | Unstable<br>Macro-<br>emulsion |      |
| 2             | Neat Oleic<br>Acid/Oleic<br>Acid 100%<br>neutralized<br>with Mono-<br>ethanolamine | 93.0             | 1<br>(0.89/0.11)     | 0.026                                | 5                                        | 0.0 | 3.0                 | ≥10000 | Stable<br>Macro-<br>emulsion   |      |

40 Samples 1 and 2 were each prepared using 1% volume of surfactant package, each having an HLB of 3.0. These samples were prepared having 5% volume of water (310 ppm brine), and each was prepared without the use of a cosolvent. Sample 1 was prepared using moderate turbulence, mixing with a Rushton impulser coupled to a Heidolph motor, which 45 provided an average mechanical power or energy dissipation rate of 1 W/kg, for 2 minutes (maximum local value of 100 W/kg). The result was an unstable macroemulsion. Sample 2 was prepared utilizing high turbulence, mixing with an Ultraturrax mixer (rotor-stator mixer), which provided mechanical power or energy dissipation rate of 10,000 W/kg 50 for 2 minutes. This resulted in a stable macroemulsion. Thus, the mixing intensity of the present invention is critical in obtaining a stable macroemulsion.

Table 15 shows results obtained with Samples 3, 4, 5 and 6, and further illustrates the criticality of mixing intensity in accordance with the present invention.

TABLE 15

| Sample<br>No. | Surfactant                            | Vol. %<br>Diesel | Vol. %<br>Surfactant | Vol. %<br>Mono-<br>ethanol-<br>amine | Deionized<br>Water<br>(310 ppm<br>Brine) |     | Vol. %<br>n-Hexanol | HLB | Mix.<br>Inten.<br>W/Kg         | Obs. |
|---------------|---------------------------------------|------------------|----------------------|--------------------------------------|------------------------------------------|-----|---------------------|-----|--------------------------------|------|
|               |                                       |                  |                      |                                      | 10                                       | 0.0 |                     |     |                                |      |
| 3             | Neat Oleic<br>Acid/Oleic<br>Acid 100% | 87.9             | 2.0<br>(1.77/0.23)   | 0.05                                 | 10                                       | 0.0 | 3.0                 | 1   | Unstable<br>Macro-<br>emulsion |      |

TABLE 15-continued

| Sample No. | Surfactant                                                        | Vol. % Diesel | Vol. % Surfactant  | Vol. % Monoethanolamine | Vol. % Deionized Water (310 ppm Brine) | Vol. % n-Hexanol | HLB | Mix. Inten. W/Kg | Obs.                   |
|------------|-------------------------------------------------------------------|---------------|--------------------|-------------------------|----------------------------------------|------------------|-----|------------------|------------------------|
| 4          | neutralized with Monoethanolamine                                 | 87.9          | 2.0<br>(1.77/0.23) | 0.05                    | 10                                     | 0.0              | 8.0 | ≥10000           | Stable Macroemulsion   |
| 5          | Neat Oleic Acid/Oleic Acid 100% neutralized with Monoethanolamine | 87.8          | 2.0<br>(1.01/0.99) | 0.22                    | 10                                     | 0.0              | 9.5 | 1                | Unstable Macroemulsion |
| 6          | Neat Oleic Acid/Oleic Acid 100% neutralized with Monoethanolamine | 87.8          | 2.0<br>(1.01/0.99) | 0.22                    | 10                                     | 0.0              | 9.5 | ≥10000           | Stable Macroemulsion   |

Samples 3 and 4 were prepared utilizing the same surfactant package having an HLB of 3.0, and a vessel-averaged mixing intensity of 1 W/kg provided an unstable macroemulsion while a mixing intensity of 10,000 W/kg produced a stable macroemulsion. Samples 5 and 6 were prepared utilizing a different surfactant package having an HLB of 9.5, and similar results were obtained. Thus, the method of the present invention can provide a stable macroemulsion at HLB values of 3 and 9.5.

Table 16 sets forth results obtained utilizing a different surfactant package. This surfactant package included 1.2% volume sorbitan ester monooleate (HLB=4.3) and 0.05% volume oleic acid 100% neutralized with monoethanolamine and had a resulting HLB of 3.

TABLE 16

| Sample No. | Surfactant                                                                  | Vol. % Diesel | Vol. % Surfactant  | Vol. % Monoethanolamine | Vol. % Deionized Water (310 ppm Brine) | Vol. % n-Hexanol | HLB | Mixing Intensity W/Kg | Obs.                   |
|------------|-----------------------------------------------------------------------------|---------------|--------------------|-------------------------|----------------------------------------|------------------|-----|-----------------------|------------------------|
| 7          | Sorbitan ester monooleate/Oleic Acid 100% neutralized with monoethanolamine | 93.7          | 1.25<br>(1.2/0.05) | 0.01                    | 5                                      | 0.0              | 3   | 1                     | Unstable Macroemulsion |
| 8          | Sorbitan ester monooleate/Oleic Acid 100% neutralized with monoethanolamine | 93.7          | 1.25<br>(1.2/0.05) | 0.01                    | 5                                      | 0.0              | 3   | ≥10000                | Stable Macroemulsion   |

## 25

The emulsions prepared for Samples 7 and 8 were 5% water emulsions, and Sample 7 prepared utilizing a vessel-averaged mixing intensity of 1 W/kg resulted in an unstable macroemulsion. Sample 8 prepared in accordance with the present invention at a mixing intensity of 10,000 W/kg, however, resulted in a stable macroemulsion.

Table 17 sets forth results obtained utilizing two additional surfactant packages for 10% volume of water emulsions.

TABLE 17

| Sample No. | Surfactant                                                                   | Vol. % Diesel | Vol. % Surfactant | Vol. % Mono-ethanolamine | Vol. % Deionized Water (310 ppm Brine) | Vol. % n-Hexanol | HLB | Mix. Inten. W/Kg | Obs.                    |
|------------|------------------------------------------------------------------------------|---------------|-------------------|--------------------------|----------------------------------------|------------------|-----|------------------|-------------------------|
| 9          | Sorbitan ester monooleate/ Oleic Acid 100% neutralized with monoethanolamine | 87.5          | 2.5 (2.4/0.1)     | 0.02                     | 10                                     | 0.0              | 3.0 | 1                | Unstable Macro-emulsion |
| 10         | Sorbitan ester monooleate/ Oleic Acid 100% neutralized with monoethanolamine | 87.5          | 2.5 (2.0/0.5)     | 0.02                     | 10                                     | 0.0              | 3.0 | ≥10000           | Stable Macro-emulsion   |
| 11         | Sorbitan ester monooleate/ Oleic Acid 100% neutralized with monoethanolamine | 87.3          | 2.5 (1.6/0.9)     | 0.2                      | 10                                     | 0.0              | 9.5 | 1                | Unstable Macro-emulsion |
| 12         | Sorbitan ester monooleate/ Oleic Acid 100% neutralized with monoethanolamine | 87.3          | 2.5 ((1.6/0.9))   | 0.2                      | 10                                     | 0.0              | 9.5 | ≥10000           | Stable Macro-emulsion   |

Samples 9 and 10 were both prepared utilizing surfactant packages including 2.4% volume sorbitan ester monooleate and 0.1% volume oleic acid 100% neutralized with monoethanolamine. This surfactant had an HLB of 3.0. Sample 9 was prepared utilizing a vessel-averaged mixing intensity of 1 W/kg, and an unstable macroemulsion resulted. Sample 10 was prepared utilizing mixing intensity in accordance with the present invention of 10,000 W/kg, and a stable macroemulsion resulted.

Samples 11 and 12 show similar results when the surfactant package is modified to have an HLB of 9.5.

Thus, as demonstrated above, Diesel fuel macroemulsions can be prepared in accordance with the present invention at

greatly reduced surfactant concentrations and having HLB values of between 3 and 10. Further, solvents or cosolvents are not needed to form a stable macroemulsion.

## 26

## EXAMPLE 5

Water incorporation is achieved in accordance with the present invention, in both microemulsions and macroemul-

5

sions, by adjusting the hydrophilic to lipophilic balance of the surfactant package and the mixing conditions. This versatility allows the development of the most cost effective fuel formations, depending on current market needs, based upon the synergistic effect between surfactant concentration and energy dissipation rate in the mixing process. This example demonstrates such different formulations which can be prepared.

10 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9

27

As shown, Sample 1 was prepared using 7% volume of the surfactant package to provide an HLB of 8.9, with 10% volume of water and 1% volume of n-Hexanol cosolvent. The mixing intensity was high, that is 10,000 W/kg, and a stable microemulsion resulted. Sample 2 was prepared utilizing the same conditions, but 2% volume of the surfactant package and no cosolvent whatsoever. This resulted in a stable mac-

28

roemulsion. Thus, through adjusting the amounts of surfactant and cosolvent, microemulsion and macroemulsion can selectively be prepared to meet particular market needs.

5 Table 19 sets forth a similar comparison utilizing a surfactant package of oleic acid 100% neutralized with monoethanolamine and sorbitan ester trioleate (HLB=1.8).

TABLE 19

| Sample No. | Surfactant                                                                   | Vol. % Diesel | Vol. % Surfactant | Vol. % Mono-ethanol-amine | Vol. % Deionized Water (310 ppm Brine) | Vol. % n-Hexanol | Mix. HLB | Inten. W/Kg | Obs.                  |
|------------|------------------------------------------------------------------------------|---------------|-------------------|---------------------------|----------------------------------------|------------------|----------|-------------|-----------------------|
| 3          | Oleic Acid 100% neutralized with mono-ethanolamine/ Sorbitan ester trioleate | 81.07         | 6 (2/4)           | 0.43                      | 10                                     | 2.5              | 7.2      | ≥10000      | Micro-emulsion        |
| 4          | Oleic Acid 100% neutralized with mono-ethanolamine/ Sorbitan ester trioleate | 87.4          | 2 (0.62/1.9)      | 0.14                      | 10                                     | 0.0              | 7.2      | ≥10000      | Stable Macro-emulsion |

These samples were also prepared containing 10% volume of water, and the surfactant package had an HLB of 7.2. 30 Further, both samples were prepared using a mixing intensity of 10,000 W/kg. Sample 3 included 6% volume of the surfactant package and 2.5% volume of n-Hexanol cosolvent, and a stable microemulsion resulted. Sample 4 was prepared utilizing 2.5% volume of the surfactant package and no cosolvent and a stable macroemulsion resulted. Thus, as with Table 18, desirable microemulsions and macroemulsions can be obtained to meet market needs by adjusting the amount of surfactant and cosolvent to be used.

35

## EXAMPLE 6

45 This example demonstrates the chemical modification of a surfactant package in accordance with the present invention so as to provide an additional property to the final emulsion, in this case for enhancing auto ignition properties of the microemulsion.

50 A nitro-olefin derivate of oleic acid was prepared for use as a surfactant component as follows. A flask containing a solution of oleic acid (10 g; 0.035 moles) in 1,2-dichloroethane (200 ml) was evacuated. Then, the flask was filled with nitrogen monoxide gas and the solution was stirred under atmospheric pressure of nitrogen monoxide at room temperature for 3 hours. The nitrogen monoxide was released, and the solvent was removed in a vacuum so as to provide a nitro-olefin derivate of oleic acid (60%) which was identified by <sup>1</sup>H NMR, <sup>13</sup>C NMR and IR analysis.

55 60 A microemulsion of 10% volume water in Diesel fuel was prepared with sample 1 using a surfactant package including oleic acid 50% neutralized with monoethanolamine so as to provide an HLB of 3, and with Sample 2 prepared utilizing nitro olefin derivate of oleic acid 50% neutralized with monoethanolamine to provide an HLB of 3.0. Table 20 sets forth analysis results for both samples.

TABLE 20

| Sample No. | Surfactant                                                                | Vol. % Diesel | Vol. % Surfactant | Vol. % Monoethanolamine | Vol. % Deionized Water (310 ppm Brine) | Vol. % n-Hexanol | Mix. Inten. W/Kg | Cetane Number |
|------------|---------------------------------------------------------------------------|---------------|-------------------|-------------------------|----------------------------------------|------------------|------------------|---------------|
| 1          | Oleic Acid 50% neutralized with monoethanolamine                          | 79            | 9                 | 1                       | 10                                     | 1                | 1                | 41.6          |
| 2          | Nitro olefin derivate of oleic acid 50% neutralized with monoethanolamine | 79            | 9                 | 1                       | 10                                     | 1                | 1                | 45.2          |

As shown in Table 20, the microemulsions were prepared having 9% volume of the surfactant package and using 1% volume of n-Hexanol cosolvent, at a vessel-averaged mixing intensity of 1 W/kg. Each sample resulted in a stable microemulsion. Note, however, that Sample 1 had a cetane number of 41.6, while Sample 2 prepared utilizing the chemically modified surfactant package had an increased cetane number of 45.2. Thus, it is clear that in accordance with the present invention, the oleic acid surfactant component can be chemically modified, for example to incorporate a nitro-group, so as to improve the functionality of the surfactant package and the resulting microemulsion.

#### EXAMPLE 7

This example demonstrates excellent results of use of an emulsion as an engine fuel in accordance with the present invention, as compared to the base hydrocarbon used as fuel. As will be demonstrated below, the emulsion of the present invention shows consistent reduction of  $\text{NO}_x$  at all operating regimes, reduction in particulate matter emissions, particularly at high partial loads, significant reduction in exhaust gas opacity under free acceleration conditions, reduced combustion duration by controlled rate of pressure rise and diffusion burning rates, adequate fuel stability in engine injection system components and improve fuel lubricity for protection of injection system components.

This example was conducted using a commercial Diesel engine installed on a test bench. The Diesel engine characteristics included 6 cylinders, direct injection, turbo charged, compression ratio: 17.5:1, displacement 5.78 liters, maximum torque: 328 Nw-m at 1800 rpm, maximum power: 153 Hp and 2500 rpm.

Steady state tests were conducted. Also, in-cylinder analysis was carried through combustion chamber and injection event observation based on piezoelectric pressure transducer measurements versus crank angle positions. Exhaust emission measurements were taken by transporting gaseous emissions to analyzer measurement cells through heated sample lines.  $\text{NO}_x$  measurements were obtained using a chemiluminescence analyzer. The hydrocarbon measurement technique was a heated flame ionization detector. CO measurement was obtained utilizing a non-dispersive infrared analyzer. Transient tests were also conducted including integrated mass emission determination of carbonaceous matter (C) using a modified US heavy duty transient cycle (1200 sec duration, rpm vs. low operation, motoring segments not applied, engine at idle). The measurement technique included analysis of the extinction of infrared radiation at specific wavelengths, with

interference filters at 3.95 microns for carbon. Exhaust opacity during free acceleration test was measured using partial flow opacimeter (HSU).

Table 21 below sets forth the fuel properties for testing a base Diesel fuel and a microemulsion prepared utilizing this fuel in accordance with the present invention.

TABLE 21

| Characteristics            | Base Fuel | Prototype                             |
|----------------------------|-----------|---------------------------------------|
| Oleic acid (% v)           | —         | 9.0                                   |
| Monoethanolamine (% v)     | —         | 1.0                                   |
| n-Hexanol (% v)            | —         | 1.0                                   |
| Water (% v)                | —         | 10.0                                  |
| Viscosity @ 40° C. (cSt)   | 3.07      | 5.45                                  |
| Lubricity (microns)        | 3.30      | 260                                   |
| ASTM D-6079 HFRR @60° c.   |           |                                       |
| Aromatic (% w)             | 18.4      | 14.1                                  |
| Density @ 15.6° C. (mg/ml) | 0.839     | 0.863                                 |
| Cetane number              | 47.3      | 46.9                                  |
|                            |           | (with the addition of cetane improver |

Based upon the cylinder pressure versus crank angle measurements for the operating condition of 1600 rpm and 157.5 pounds-ft of torque (50% of partial load), as indicated in FIG. 2, a heat release calculation was performed in the closed portion of the thermodynamic cycle to determine fuel combustion details. The results of this calculation are shown in Table 22.

TABLE 22

| Variable                                               | Base fuel | Prototype |
|--------------------------------------------------------|-----------|-----------|
| Start of injection (° before top dead center)          | 9.0       | 8.0       |
| Ignition delay (°)                                     | 4.8       | 6.4       |
| Crankangle for 90% of the injected fuel energy release | 38.0      | 35.2      |

It can be inferred that considering similar conditions of start of injection, longer ignition delay and faster combustion rate during diffusion burning (similar total energy release for smaller number of crank angles), strongly determines the performance for the microemulsion of the present invention as compared to the base fuel.

A qualitative explanation can be devised considering (a) different localized temperature regimes due to extended cold fuel jet and energy required for water vaporization and heating; (b) an enhanced fuel-air mixing mechanism; both of

31

which are related to water being present in the injected Diesel fuel droplets. It is believed that the incorporation of the water phase promotes additional breakup and dispersion with relatively wider spray angles and higher air entrainment during the fuel atomization process. Oxygen contribution due to accessibility, soot formation inhibition and mixture leaning are also potential acting mechanisms.

Fuel stability at engine conditions was observed and is satisfactory based upon the absence of fuel/water separation in the return fuel line for excess and leak back flow from injectors. FIG. 3 shows  $\text{NO}_x$  exhaust gas emission rates for both fuels, and the microemulsion of the present invention shows consistent reduction of  $\text{NO}_x$  at all operating regimes.

Particulate matter emissions were reduced at high loads as shown by consideration of accumulated exhaust gas carbon mass during transient engine operation. The carbon mass emissions between the microemulsion of the present invention and the base fuel began to differ significantly after applying high partial loads to the engine in transient operation. This is also illustrated in FIG. 4.

Significant reductions of exhaust gas opacity under free acceleration conditions are also illustrated in FIG. 5. This reduction in opacity also out-performed several other fuel reformulation possibilities which have been previously tested on this same engine, namely, lower aromatics, higher cetane, and lower sulfur fuel as compared to prototype fuel.

It was also possible to achieve reduced ignition delays among different water emulsified fuels, which will result in improved engine performance, by controlled rate of pressure rise due to varying the amount of surfactant package and modifying the real logical properties of the fuel in the spray plume.

Thus, the microemulsion of the present invention is clearly an advantageous alternative to the base fuel.

#### EXAMPLE 8

As set forth above, the present invention also provides for tuning of a fuel to specific combustion chamber environment conditions. This is accomplished by adjusting the chemistry of the fuel and its physico-chemical and rheologic properties. To illustrate this, a second microemulsion fuel formulation was prepared and compared to the microemulsion prepared in Example 7. Table 23 lists the characteristics of the Example 7 microemulsion and microemulsion 2, each of which incorporates 10% volume of water. Microemulsion 2 was prepared utilizing a lower concentration of the surfactant package and different mixing intensity conditions, specifically, continuous production using a static mixer in turbulent flow, with energy dissipation rate per unit mass of mixture in the mixer of not less than 100 W/kg. Both fuels were also compared to the base fuel as described in Table 21.

TABLE 23

| Characteristics                        | Prototype                              | Prototype 2 |
|----------------------------------------|----------------------------------------|-------------|
| Oleic acid (% v)                       | 9.0                                    | 7.0         |
| Monoethanolamine (% v)                 | 1.0                                    | 0.7         |
| n-Hexanol (% v)                        | 1.0                                    | 0.7         |
| Water (% v)                            | 10.0                                   | 10.0        |
| Viscosity @ 40° C. (cSt)               | 5.45                                   | 3.95        |
| Aromatic (% v)                         | 14.1                                   | 14.6        |
| Density @ 15.6 C. (mg/ml)              | 0.863                                  | 0.852       |
| Cetane number                          | 46.9                                   | 46.5        |
| (with the addition of cetane improver) | (with the addition of cetane improver) |             |

32

As shown microemulsion 2 has reduced viscosity, slightly increased aromatics content and slightly reduced base cetane number.

Table 24 below sets forth engine performance comparison on the same engine as described in Example 7 for both the microemulsion of Example 7 and microemulsion 2 prepared as outlined in Table 23.

TABLE 24

| Engine performance                                                 | Prototype | Prototype 2 |
|--------------------------------------------------------------------|-----------|-------------|
| NOx emissions (% of difference versus Base Fuel)                   | -12.9     | -12.0       |
| Engine operating condition:<br>1600 rpm @ 252.0 lbf·ft             | -20.8     | -35.1       |
| Soot emissions (% of difference versus Base Fuel)                  |           |             |
| Engine operating condition:<br>1600 rpm @ 252.0 lbf·ft             | -0.3      | +3.5        |
| Fuel conversion efficiency (% of difference versus Base Fuel)      |           |             |
| Engine operating condition:<br>1600 rpm @ 252.0 lbf·ft             | -13.2     | -7.3        |
| Maximum engine brake horsepower (% of difference versus Base Fuel) |           |             |
| Engine operating condition:<br>(WOT) @ 2500 rpm                    |           |             |

As shown, similar reductions in  $\text{NO}_x$  emissions were accomplished with both emulsions. This is believed to be related to the equivalent water content in both fuels.

However, soot emissions are improved utilizing microemulsion 2. Fuel conversion efficiency of fuel of microemulsion 2 is also improved and the power difference as compared to the base fuel is reduced from negative 13.2% to negative 7.3%. These results clearly indicate an improved engine performance which is accomplished by adjusting the physical chemical and rheological properties of the fuel during water incorporation.

#### EXAMPLE 9

40 This example is presented so as to demonstrate a synergism between oleic acid surfactant and the salt of oleic acid which is generated with monoethanolamine according to the invention.

45 FIG. 6 illustrates interfacial tension between water and hydrocarbon phases utilizing a surfactant package which includes 2% volume of oleic acid and varying amounts of monoethanolamine. As illustrated in this figure, there is a concentration interval of monoethanolamine (MEA) wherein ultra low interfacial tensions are obtained. When this point is reached, the system is emulsified spontaneously in the measurement equipment. In this concentration interval of MEA, there is found adsorbed in the interface Diesel/water the two surfactants, that is, oleic acid and oleate ions. In the extreme 50 regions of FIG. 6, that is to say, at the low and high concentrations of MEA, are found the oleic acid and the oleate ions individually adsorbed in the interface, and the interfacial tensions are the highest. This is believed to be due to the following.

55 When the oleic acid dissolved in the Diesel fuel enters into contact with the MEA and the water, there occurs an acid/base reaction in the interface Diesel/water to give rise to the oleate ions. The oleic acid as well as the oleate ions are adsorbed in the interface Diesel/water due there infinity to the water as the oil. At intermediate concentrations of MEA (0.04-0.3% volume), the oleic acid is appreciably ionized so as to provide oleate ions, and the interface Diesel/water will be covered by

## 33

both oleate ions and oleic acid. In this zone, synergistic interfacial tension is illustrated, since the interfacial tension is lower than that obtained from either of the surfactants individually.

It should be appreciated that a water-in-hydrocarbon emulsion has been provided which exhibits advantageous characteristics as compared to conventional fuels, and that methods for advantageously forming such emulsions have also been provided.

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

What is claimed:

1. A method for forming a stable water in liquid hydrocarbon microemulsion, comprising the steps of:

providing a liquid hydrocarbon phase;

providing a water phase;

providing a surfactant package having an HLB of between about 6 and about 10 and having a lipophilic component having an HLB of between about 1 and about 8 and a hydrophilic component having an HLB of between about 10 and about 18, wherein said surfactant package further includes a functional group for improving performance of said stable microemulsion as a combustible fuel, said functional group being different from said lipophilic component and said hydrophilic component and selected from the group consisting of nitrogen groups, ketones, hydroxy and epoxy groups, and mixtures thereof; and

mixing said liquid hydrocarbon phase, said water phase and said surfactant package at a ratio by volume of said water phase to said surfactant of at least about 1, with said water phase in an amount of between about 5% and about 15% volume with respect to volume of said microemulsion, and at a mixing intensity of at least about 1 W/kg, so as to provide a stable water in liquid hydrocarbon microemulsion wherein said lipophilic component and said hydrophilic component are present at an interface between said water phase and said liquid hydrocarbon phase, and wherein said lipophilic component comprises a nitro-olefin derivate of oleic acid obtained by using nitrogen monoxide to modify the oleic acid.

2. The method of claim 1, wherein said functional group is a nitrogen oxide group.

3. A method for forming a stable water and liquid hydrocarbon macroemulsion, comprising the steps of:

providing a liquid hydrocarbon phase;

providing a water phase;

providing a surfactant package having an HLB of between about 3 and about 10 and having a lipophilic component having an HLB of between about 1 and 8 and a hydrophilic component having an HLB of between about 10 and about 18, wherein said surfactant package further includes a functional group for improving performance of said stable macroemulsion as a combustible fuel, said functional group being different from said lipophilic component and said hydrophilic component and selected from the group consisting of nitrogen groups, ketones, hydroxy and epoxy groups, and mixtures thereof; and

mixing said liquid hydrocarbon phase, said water phase and said surfactant package at a ratio by volume of said

## 34

water phase to said surfactant of at least about 1, with said water phase in an amount of between about 5% and about 15% volume with respect to volume of said macroemulsion, and at a mixing intensity of at least about 10,000 W/kg, so as to provide a stable water in liquid hydrocarbon macroemulsion wherein said lipophilic component and said hydrophilic component are present at an interface between said water phase and said liquid hydrocarbon phase, and wherein said lipophilic component comprises a nitro olefin derivate of oleic acid obtained by using nitrogen monoxide to modify the oleic acid.

4. The method of claim 3, wherein said functional group is a nitrogen oxide group.

5. A stable water-in-liquid hydrocarbon microemulsion, comprising a water phase, a liquid hydrocarbon phase and a surfactant package having an HLB of between about 6 and about 10 and having a lipophilic component having an HLB of between about 1 and about 8 and a hydrophilic component having an HLB of between about 10 and about 18, wherein said surfactant package further includes a functional group for improving performance of said stable microemulsion as a combustible fuel, said functional group being different from said lipophilic component and said hydrophilic component and selected from the group consisting of nitrogen groups, ketones, hydroxy and epoxy groups, and mixtures thereof; wherein said water phase and said surfactant package are present at a ratio by volume of said water phase to said surfactant package of at least about 1, wherein said water phase is present in an amount between about 5% and about 15% volume with respect to said microemulsion, and wherein said lipophilic component and said hydrophilic component are present at an interface between said water phase and said liquid hydrocarbon phase, and wherein said lipophilic component comprises a nitroolefin derivate of oleic acid obtained by using nitrogen monoxide to modify the oleic acid.

6. The microemulsion of claim 5, wherein said functional group is a nitrogen oxide group.

7. A stable water-in-liquid hydrocarbon macroemulsion, comprising a water phase, a liquid hydrocarbon, and a surfactant package having an HLB of between about 3 and about 10 and having a liquid lipophilic component having an HLB of between about 1 and about 8 and a hydrophilic component having an HLB of between about 10 and about 18; and

wherein said surfactant package further includes a functional group for improving performance of said stable macroemulsion as a combustible fuel, said functional group being different from said lipophilic component and said hydrophilic component and selected from the group consisting of nitrogen groups, ketones, hydroxy and epoxy groups, and mixtures thereof, wherein said water phase and said surfactant package are present at a ratio by volume of said water phase to said surfactant package of at least about 1, wherein said water phase is present in an amount between about 5% and about 15% volume with respect to said macroemulsion, and wherein said lipophilic component and said hydrophilic component are present at an interface between said water phase and said liquid hydrocarbon phase, and wherein said lipophilic component comprises a nitroolefin derivate of oleic acid obtained by using nitrogen monoxide to modify the oleic acid.

8. The macroemulsion of claim 7, wherein said functional group is a nitrogen oxide group.

## 35

9. A method for forming a stable water in liquid hydrocarbon microemulsion, comprising the steps of:

providing a liquid hydrocarbon phase;

providing a water phase;

providing a surfactant package having an HLB of between about 6 and about 10 and having a lipophilic component having an HLB of between about 1 and about 8, a hydrophilic component having an HLB of between about 10 and about 18 and a functional group for improving performance of said stable microemulsion as a combustible fuel, wherein said functional group is a nitrogen oxide group; and

mixing said liquid hydrocarbon phase, said water phase and said surfactant package at a ratio by volume of said water phase to said surfactant of at least about 1, with said water phase in an amount of between about 5% and about 15% volume with respect to volume of said microemulsion, and at a mixing intensity of at least about 1 W/kg, so as to provide a stable water in liquid hydrocarbon microemulsion wherein said lipophilic component and said hydrophilic component are present at an interface between said water phase and said liquid hydrocarbon phase, wherein said lipophilic component comprises a nitroolefin derivate of oleic acid obtained by using nitrogen monoxide to modify the oleic acid.

10. A method for forming a stable water and liquid hydrocarbon macroemulsion, comprising the steps of:

providing a liquid hydrocarbon phase;

providing a water phase;

providing a surfactant package having an HLB of between about 3 and about 10 and having a lipophilic component having an HLB of between about 1 and 8 and a hydrophilic component having an HLB of between about 10 and about 18 and a functional group for improving performance of said stable microemulsion as a combustible fuel, wherein said functional group is a nitrogen oxide group; and

mixing said liquid hydrocarbon phase, said water phase and said surfactant package at a ratio by volume of said water phase to said surfactant of at least about 1, with said water phase in an amount of between about 5% and about 15% volume with respect to volume of said macroemulsion, and at a mixing intensity of at least about 10,000 W/kg, so as to provide a stable water in liquid hydrocarbon macroemulsion wherein said lipophilic

## 36

component and said hydrophilic component are present at an interface between said water phase and said liquid hydrocarbon phase, wherein said lipophilic component comprises a nitro olefin derivate of oleic acid obtained using nitrogen monoxide to modify the oleic acid.

11. A stable water-in-liquid hydrocarbon microemulsion, comprising a water phase, a liquid hydrocarbon phase and a surfactant package having an HLB of between about 6 and about 10 and having a lipophilic component having an HLB of between about 1 and about 8 and a hydrophilic component having an HLB of between about 10 and about 18 and a functional group for improving performance of said stable microemulsion as a combustible fuel, wherein said functional group is a nitrogen oxide group, wherein said water phase and said surfactant package are present at a ratio by volume of said water phase to said surfactant package of at least about 1, wherein said water phase is present in an amount between about 5% and about 15% volume with respect to said microemulsion, and wherein said lipophilic component and said hydrophilic component are present at an interface between said water phase and said liquid hydrocarbon phase, wherein said lipophilic component comprises a nitroolefin derivate of oleic acid obtained by using nitrogen monoxide to modify the oleic acid.

12. A stable water-in-liquid hydrocarbon macroemulsion, comprising a water phase, a liquid hydrocarbon, and a surfactant package having an HLB of between about 3 and about 10 and having a liquid lipophilic component having an HLB of between about 1 and about 8 and a hydrophilic component having an HLB of between about 10 and about 18 and a functional group for improving performance of said stable microemulsion as a combustible fuel, wherein said functional group is a nitrogen oxide group, wherein said water phase and said surfactant package are present at a ratio by volume of said water phase to said surfactant package of at least about 1, wherein said water phase is present in an amount between about 5% and about 15% volume with respect to said macroemulsion, and wherein said lipophilic component and said hydrophilic component are present at an interface between said water phase and said liquid hydrocarbon phase, wherein said lipophilic component comprises a nitroolefin derivate of oleic acid obtained by using nitrogen monoxide to modify the oleic acid.

\* \* \* \* \*